

## UNITED STATES PATENT OFFICE

2,183,587

## EXOTHERMIC MIXTURE

Ferdinand Racen, St. Louis, Mo., and Walter M. Bruner, New Haven, Conn., assignors to W. G. Shelton Company, St. Louis, Mo., a corporation of Missouri

No Drawing. Application December 4, 1936,  
Serial No. 114,204

## 16 Claims. (Cl. 44—3)

This invention relates to an exothermic chemical composition which, when moistened with water, or aqueous liquid, spontaneously evolves a controllable quantity of heat and may be used in pads or envelopes of suitable construction for various purposes, such as therapeutic heating pads, hair-waving heating pads, and the like.

The heat evolving properties of the chemical composition depend upon the principle of oxidation-reduction which is known to be a highly exothermic chemical process, and which is set in action by the moistening of the chemical composition with the liquid. Under certain operating conditions it is essential that the reactions conform closely to well defined requirements in order that best results be secured. For example, in a hair waving pad when the mixture is moistened the resulting temperature should rise to the boiling point of the liquid in from thirty seconds to three minutes, and this temperature should be sustained for about five minutes and then increased about 2° to 10° C. in one to three minutes, and thereafter drop quite rapidly to about 50° C. when the pad may be handled by the operator without discomfort.

It is necessary that the water vapor evolved during the active heating period of the composition be emitted slowly and gently to avoid burning the scalp by strong jets of steam. It is also necessary that the composition be of a stable character, so that pads several months old will commence heating within two or three minutes after moistening.

The objects of the invention are to fulfill the above mentioned requirements and to avoid the disadvantages expressed or implied.

The composition consists primarily of a mixture of metals with other ingredients which in the presence of water aid in the oxidation of the metallic mixture. Aluminum is to be preferred as the principal metallic ingredient because of its cheapness, convenience, and the high heat of formation of its compounds, although iron, magnesium, zinc, cadmium and other metals may be used. In practice it is found that the composition is improved by the use of a secondary metal, positioned lower in the electromotive series of metals, such as copper, zinc, tin, bismuth, antimony, lead, mercury, arsenic, and active alloys of the same containing sufficient of the named metal to be substantially as active as the named metal. The purpose of these metals is to supply heat by means of their oxidation. We have found that the duration of the heating period may be

easily controlled by means of the proportion of these metals present in the composition.

As an oxidizing agent such highly oxygenated compounds as potassium dichromate, barium peroxide, benzoyl peroxide, potassium permanganate, ammonium persulfate, sodium perborate, magnesium perchlorate, and the like, may be used. However, because of solubility characteristics, economy, and particularly because of the highly oxidizing decomposition products which are formed when it is acidified, potassium chlorate is one of the most convenient oxidizing agents to use.

We find that the proportion of this ingredient has a pronounced effect upon the course of the heating period, particularly in determining the point of rise above the boiling temperature of water and the rate of final cooling.

An acidic substance which produces acid by hydrolysis, and which contains a metal displaceable by the principal metal reducing agent, serves not only to act as a source of acid to decompose the oxidizing agent but also to supply quickly available heat by means of a displacement reaction. The proportion and properties of this ingredient regulates the time necessary to reach the boiling temperature of water. This substance may be cupric sulfate, cupric nitrate, cuprous chloride, cupric formate, cupric tartrate, cupric chlorate, cupric lactate, cupric salicylate, cupric sulfite, cupric phosphate, cupric acetate, cuprous bromide, cuprous sulfite, cuprous iodide, cuprous ammonium iodide, and the corresponding salts of iron, cobalt, nickel, tin, bismuth, mercury, arsenic, antimony, and lead. However, it is found that greater stability of the composition will result if the salts of relatively low solubility such as cuprous chloride and cupric tartrate are selected.

In place of the above named source of an acidic media which produces a preponderance of hydrogen ions, certain soluble solid organic acids may be used and their very slight tendency to absorb water from the atmosphere helps minimize undesirable decomposition of the ingredients due to the absorption of moisture from the atmosphere. Another advantage of the weak solid organic acids is that their partial wetting by means of small amounts of water in the surrounding atmosphere has less corrosive and deleterious effects on the other ingredients, whereas the hydrolysis of acidic inorganic salts like cuprous chloride may result in the formation of strong mineral acids which attack other active ingredients of the mixture. Acidic substances which may be used for this purpose are oxalic acid, tartaric acid, adipic acid,

benzoic acid, cinnamic acid, isocinnamic acid, uric acid, maleic acid, oxamic acid, pimelic acid, phthalic acid, phthalic anhydride, salicylic acid, tannic acid, toluic acid, and the like. The functioning of the acid or mixture of acids in the mixture is found to depend upon the polarity, solubility, and neutral equivalent, all of which are closely related as far as this problem is concerned. For example, an exothermic mixture containing benzoic acid, which is an acid of lower water solubility, higher neutral equivalent and lower polarity than tartaric acid, will require longer to attain the boiling temperature of water than one containing the latter acid in the same proportion.

15 The above indicates the nature and specific embodiments of the essential ingredients in the composition. Others may be added to control the evolution of heat, increase the shelf life of the finished product, for economy, or for some other 20 reason.

25 Certain oxides like cuprous and cupric oxides appear to be valuable addition agents because they accelerate the evolution of heat, evidently by means of replacement reactions. Such oxides are, however, not essential components.

An additional function of such elements is to stabilize the mixture because they are relatively inert when subjected to atmospheric moisture only, although becoming active when combining 30 with the acidic media produced by the addition of a substantial quantity of water to the mixture.

The addition of a small proportion of mineral oil is beneficial in retarding the speed of chemical action when the boiling temperature of water 35 is reached, and in increasing protection from atmospheric deterioration. The oil appears to form a thin protective film over the surface of the ingredients, thereby slowing down the evolution of water vapor. The so-called drying oils such as 40 linseed and China-wood oils are very effective, and in addition they aid the stability of the composition probably by the removal of free oxygen from the atmosphere and occluded on the surface of the active ingredients.

45 Certain desiccating agents, such as calcium sulfate or magnesium carbonate, may be added to preserve the dryness of the packaged mixture. This is also aided by preliminary oven-drying of the mixture before packing.

50 As a diluent for the active ingredients, to aid in protecting the active ingredients from the deleterious effects of the atmosphere, to reduce the cost of the composition, and to aid in securing the proper quantity of heat from each pad, we may use pumice, kaolin, kieselguhr, silica, chalk, 55 calcium sulfate, gypsum, or any other cheap chemically inert material.

The following is an example of a composition which we find to be satisfactory:

|                       | Grams |
|-----------------------|-------|
| 60 Pumice             | 6.0   |
| Kaolin                | 4.0   |
| Aluminum              | 3.0   |
| Brass                 | 2.0   |
| 65 Potassium chloride | 1.5   |
| Cuprous oxide         | 0.2   |
| Cuprous chloride      | 0.6   |
| Linseed oil           | 0.2   |
| Magnesium carbonate   | 0.1   |

70 It will be perceived that the proportions of the ingredients may be quite widely varied to obtain various shapes of cooling curves.

An explanation of the chemical reactions which take place when such a mixture is moistened with 75 water is complicated by the simultaneous occur-

rence of several reactions and by the interdependence of many of the reactions. The essential processes involved, however, may be briefly summarized by the following possible equations. (The lines between some equations serve to indicate groups of reactions which theoretically follow the previous groups.)



Undoubtedly other equations expressing possible reactions could be written, although the above are sufficient to account for the behavior of the composition when moistened. It will be seen that the majority of them express oxidation-reduction or displacement reactions, both of which are known to be highly exothermic.

It will be understood that the example of a satisfactory composition upon which the foregoing equations are based suggests quantities which may be varied substantially in some instances without noticeable change in results and in other instances with changes which may be considered advantageous according to the degrees of heat produced and the time periods over which production of heat is extended. As suggestive of such variations in quantities, it is noted that the inert diluent may vary from 5 to 20 grams, the aluminum from 1 to 6 grams, the brass from 0.05 to 5 grams, the potassium chloride from 0.4 to 5 grams, the cuprous oxide from 0.05 to 4 grams, the cuprous chloride from 0.2 to 4 grams. As previously indicated, the mineral oil and magnesium carbonate may be eliminated entirely or used in quantities as stated or substantially larger.

according to the mass of the other ingredients involved.

As an example of an exothermic mix utilizing organic acid as a source of the acidic media, the following has proved satisfactory, although neither the specific ingredients named nor the proportions given need be adhered to in view of the earlier references to equivalents:

|    |                     | Grams |
|----|---------------------|-------|
| 10 | Brass               | 2.0   |
|    | Pumice              | 6.0   |
|    | Kaolin              | 4.0   |
|    | Aluminum            | 3.3   |
|    | Cuprous oxide       | 0.8   |
| 15 | Salicylic acid      | 0.8   |
|    | Raw China-wood oil  | 0.1   |
|    | Fotassium chlorate  | 2.4   |
|    | Magnesium carbonate | 0.1   |

20 The above mixture, when moistened with water, produces substantially simultaneously a number of reactions, many of which are interdependent upon each other. The most essential, although not necessarily all of the resulting actions, may 25 be summarized by the following equations, the majority of which express oxidation-reduction or displacement reactions, both of which are known to be highly exothermic:



It is obvious that numerous combinations of ingredients mentioned could be selected from the data given herein and the quantities varied to

give different results as to extent and degree of heating. All such compositions are considered as embodying the present invention when they are characterized by the presence of a metal and by the production of hydrogen or hydrogen ions or hydrochloric acid by the addition of water to an otherwise inert mass, to combine with an oxidizing agent and a substance which in an acidic media will furnish metallic ions replaceable by said metal. The mixtures may comprise two 10 metals of higher and lower electrolytic activity, respectively, and a source of acidic media of lower electrolytic activity than the metal having the higher electrode potential, or the mixture may include but a single metal and the acidic media 15 may be supplied by an aqueous solution of an organic acid.

Numerous examples of such modifications are indicated by the variations referred to in the second paragraph following the equations based upon the first formula given herein and by the reference to similar variations relative to the second formulae. The exclusive use of these and other modifications of the invention as described in the accompanying claims is contemplated. 20 25

What is claimed is:

1. A composition for producing heat by chemical action, comprising a mixture of a primary metal and a secondary metal, said primary metal being from the group of stable metals positioned above the secondary metal in the electromotive series of metals, said secondary metal being from the group of stable metals no more active than zinc and active alloys thereof, a substance stable in a dry state and capable when in solution of furnishing an acidic medium, and an oxidizing agent sufficiently active in the acidic medium and in quantity sufficient to oxidize both said primary and said secondary metal. 30 35

2. A composition as described in claim 1 in which the primary metal is selected from the group consisting of magnesium, aluminum, manganese, cadmium, zinc and active alloys of the same. 40

3. A composition as described in claim 1 in which the secondary metal is selected from the group consisting of zinc, copper, tin, bismuth, antimony, lead, mercury, arsenic, and active alloys of the same. 45

4. A composition as described in claim 1 in which the primary metal is selected from the group consisting of magnesium, aluminum, manganese, cadmium, zinc, and active alloys of the same, and the secondary metal is selected from the group consisting of zinc, copper, tin, bismuth, antimony, lead, mercury, arsenic, and active alloys of the same. 55

5. A composition as described in claim 1 in which the substance furnishing the acidic medium is selected from the group consisting of cupric sulfate, cupric nitrate, cuprous chloride, cupric formate, cupric tartrate, cupric lactate, cupric salicylate, cupric sulfite, cupric phosphate, cupric acetate, cuprous bromide, cuprous sulfite, cuprous iodide, cuprous ammonium iodide, and the corresponding salts of iron, cobalt, nickel, bismuth, mercury, tin and lead, oxalic acid, tartaric acid, adipic acid, benzoic acid, cinnamic acid, isocinnamic acid, uric acid, maleic acid, oxamic acid, pimelic acid, phthalic acid, phthalic anhydride, salicylic acid, tannic acid and toluidic acid.

6. A composition as described in claim 1 in which the oxidizing agent is selected from the group consisting of potassium chlorate, ammonium 76

nium persulfate, sodium perborate and barium peroxide.

7. A composition as described in claim 1 which includes an additional ingredient insoluble in water and normally inert under atmospheric conditions and stabilizing the mixture but being rendered active in the acidic medium, the acidic medium furnishing quickly available replaceable ions to intensify the exothermic reactions particularly in the initial stages of the processes.

8. An exothermic mixture comprising a substantial quantity of each of a primary metal and a secondary metal, said primary metal being from a group of stable metals positioned above the secondary metal in the electromotive series of metals, said secondary metal being from the group of stable metals no more active than zinc and active alloys thereof, an acidic salt of a metal of lower electrolytic activity than the first of said metals, and an oxidizing agent sufficiently active in the acidic medium and in quantity sufficient to oxidize both said primary metal and said secondary metal and reacting more readily with said primary metal than with the secondary metal.

9. An exothermic mixture comprising a substantial quantity of each of a primary metal and a secondary metal, said primary metal being from a group of stable metals positioned above the secondary metal in the electromotive series of metals, said secondary metal being from the group of stable metals no more active than zinc and active alloys thereof, an acidic salt of a metal of lower electrolytic activity than the first of said metals, and an oxidizing agent selected from the group consisting of potassium chloride, ammonium persulfate, sodium perborate and barium peroxide.

10. An exothermic mixture including an inert diluent, aluminum, potassium chloride, cuprous chloride, and brass.

11. An exothermic mixture including the following ingredients in the proportion indicated—

|                    | Grams                 |
|--------------------|-----------------------|
| Inert diluent      | approximately 5 to 20 |
| Aluminum           | do 1 to 6 5           |
| Potassium chloride | do 0.4 to 5           |
| Cuprous chloride   | do 0.2 to 4           |
| Brass              | do 0.05 to 5          |

12. An exothermic mixture including an inert diluent, aluminum, potassium chloride, cuprous chloride, brass, and cuprous oxide.

13. An exothermic mixture including the following ingredients in the proportion indicated—

|                    | Parts by weight       |
|--------------------|-----------------------|
| Inert diluent      | approximately 5 to 20 |
| Aluminum           | do 1 to 6             |
| Potassium chloride | do 0.4 to 5           |
| Cuprous chloride   | do 0.2 to 4           |
| Cuprous oxide      | do 0.05 to 4 20       |
| Brass              | do 0.05 to 5          |

14. An exothermic mixture comprising an inert diluent, aluminum, brass, potassium chloride, cuprous oxide, cuprous chloride, linseed oil, and magnesium carbonate.

15. An exothermic mixture comprising an inert diluent, approximately 10 parts by weight; aluminum, approximately 3 parts; brass, approximately 2 parts; potassium chloride, approximately 1.5 parts; cuprous oxide, approximately 0.2 part; cuprous chloride, approximately 0.6 part; mineral oil, approximately 0.2 part; and magnesium carbonate, approximately 0.2 part.

16. An exothermic mixture comprising an inert diluent, aluminum, brass, potassium chloride, salicylic acid, cuprous chloride, drying oil, and magnesium carbonate.

FERDINAND RACEN.  
WALTER M. BRUNER.